

April 1, 1947.

L. E. MOBERLY

2,418,420

PROCESS FOR IMPREGNATING CARBON BRUSHES

Filed Feb. 8, 1943



*Fig. 2.*



WITNESSES:

Edward Michaels

J. Shapoe

INVENTOR

Lawrence E. Moberly

*Frank J. Savage*  
ATTORNEY

## UNITED STATES PATENT OFFICE

2,418,420

## PROCESS FOR IMPREGNATING CARBON BRUSHES

Lawrence E. Moberly, Wilkinsburg, Pa., assignor to Westinghouse Electric Corporation, East Pittsburgh, Pa., a corporation of Pennsylvania

Application February 8, 1943, Serial No. 475,182

7 Claims. (Cl. 117—21)

1

This invention relates to the treatment of carbon bodies, more particularly in the form of brushes, with materials which render them capable of resisting dusting and wear.

In the copending patent application of H. M. Elsey, Serial No. 475,122, filed February 8, 1943, entitled "Dynamo-electric apparatus and brushes," there is disclosed a carbon electrode or brush which does not wear or dust excessively when operating against a copper current collector rotating at a high velocity under atmospheric conditions corresponding to a 40,000-foot altitude and a moisture content corresponding to a dew point of —50° C. Under such conditions, ordinary carbon brushes will wear and dust at a rapid rate and the brushes can not be used for prolonged periods of time. This has been discovered to occur at high altitudes in electrical motors and generators employed on aircraft.

It was disclosed in the aforementioned patent application that halogen compounds, particularly halide salts of metals exemplified by lead iodide, cadmium iodide, silver iodide, cadmium chloride, potassium fluoride and cadmium bromide, when applied to the brushes either by impregnation or other mode of distribution therein, will cooperate with the commutator or other current collector to reduce the wear and dusting in atmospheric conditions corresponding to those generally experienced at high altitudes.

In applying halide salts of metals to carbon electrodes, such as electrographitic brushes, in order to reduce excessive wear and dusting under high altitude conditions, it has been discovered that about 40% or more by weight of the metallic halide salt based on the weight of the brush is required for best results. This amount of such salts cannot readily be introduced into the highly compacted, finely porous, carbonaceous material in the brushes by conventional methods. Soaking the brush in saturated aqueous solutions of most metallic chlorides, iodides, fluorides and bromides, for instance, does not always provide for introducing a sufficient amount of the salt to give the optimum results since some of the salts, such for example, as lead iodide, are only slightly soluble in water.

Immersing brushes in the molten halide salt compound also has been found to be relatively unsatisfactory. The fine porosity of the brushes, in combination with the gases normally present in the pores, appears to greatly restrain penetration of the molten compound. In some cases, one hour immersion has been barely satisfactory to give an adequate amount of melted salt pene-

2

tration and deposition in the pores of the brushes. When it is considered that carbon brushes numbering millions must be treated with a predetermined amount of salt, such a process is not entirely practical.

The object of the invention is to provide a method of impregnating carbon brushes with metallic halide salts.

Other objects of the invention will, in part, be obvious, and will, in part, appear hereinafter.

For a fuller understanding of the nature and objects of this invention, reference should be had to the figures of the drawing, where:

Figure 1, partly in section, shows a schematic arrangement for carrying out the process of this invention; and

Fig. 2 is a view in elevation of a brush with halide salt deposited thereon.

According to this invention, it has been discovered that halide salts may be rapidly and efficiently applied in predetermined amount to carbon brushes by melting the salts directly upon the brushes to produce electrodes having low wear and dusting characteristics when operating under high altitude conditions.

For an example of the invention, reference should be had to the figure of the drawing in which there is illustrated a schematic arrangement of a brush impregnating apparatus 10. At the left hand of the apparatus, individual brushes 12, or carbon plates from which a number of brushes may be made, to be treated are placed on an endless conveyor 14 disposed for operation about pulleys 16 and 18 operated from a suitable source of power at a predetermined rate of travel. A receptacle 20, filled with the dry crystalline or powdered halide salt, such, for example, as lead iodide, is disposed above the brushes 12 on conveyor 14. A measuring wheel 22 having pockets of a predetermined size is fed with the lead iodide from the container 20 whereby a predetermined amount of the salt is measured out in each pocket. A mechanism (not shown) actuated by the passage of the brushes below the container 20 may be employed to turn the measuring device 22 in synchronism therewith whereby a pocket is filled for each brush. The measured quantity of salt is emptied from the pockets and is distributed by the spout 24 upon each brush 12 as the brush passes therebelow on conveyor 14. Thus, each brush 12 has applied to the upper surface thereof a measured heap or layer 26 of the lead iodide.

Instead of a powder, preformed tablets of a predetermined weight of metal halide may be

applied by a similar device to each carbon brush or plate on the conveyor.

The conveyor 14 carries the brushes with the predetermined amount of salt applied thereto into the furnace or oven 28 which is heated from a suitable source of energy to maintain a temperature well above the melting point of the salt. In the case of lead iodide, the temperature of the furnace will be about 500° C. As the brushes enter the furnace 28, the salt 26 on each brush is heated to the melting point and the molten salt rapidly penetrates the brush to thoroughly impregnate the pores thereof. For some reason not entirely known, the impregnation of the brush occurs at a rate many times greater than when the same brush is immersed in a bath of the molten compound. The high rate of penetration is entirely unexpected. Less than ten minutes in the furnace 28 is sufficient for the complete absorption of the molten compound in a carbon body of the size of 1 inch by  $\frac{1}{2}$  inch by  $\frac{1}{4}$  inch.

The heat treated salt impregnated brush 30 is carried out of the oven on the conveyor 14 where it cools rapidly and may be put in use at once. To prevent an untoward reaction of the atmosphere with the hot salt, it may be desirable to effect cooling in a nonoxidizing atmosphere maintained in a separate cooling chamber at the end of the conveyor.

In order to retain the fluid molten halide salt in contact with the upper surface of the carbon bodies during impregnation, any suitable method well known to those skilled in the art may be employed. One method that has been found to be satisfactory has been to provide a ledge or dam around the body as shown in Fig. 2. The carbon body 12 may be channeled to produce a pocket 11 defined by the ledges 13 at the sides at the upper surface. Large flat plates of carbon can be prepared, by molding or machining, with a pocket 11 in the center to provide a continuous ledge about all the edges. Smaller plates can be channeled and butted tightly against one another while on the conveyor to form a continuous trough. A layer of pitch, tar, resin, or other suitable cement can be applied between adjacent bodies to prevent molten salt leakage. The applied salt even when molten is thereby prevented from running off since it is retained in a pocket 11. In some cases separate members may be applied about the sides of carbon plates 12 to dam in the melted salt.

In order to secure a uniform distribution of metallic halide salt over the entire area of a plate 12 such as is shown in Fig. 2, the halide 26 should be evenly applied over the entire pocket 11. It has been found that upon reaching the melting point the metallic halide generally penetrates only the portions of the brush directly below it without spreading laterally to any great extent. Thus, if the heap 26 of powdered halide is applied over only a limited surface area, nonuniform impregnation may result and some brushes cut from plate 12 may contain but little impregnant.

A different method of applying an even layer of metal halide over the surface of pocket 11 is to mix the metal halide, such as lead iodide, with an easily volatilized binder such as polystyrene, coumarone-indene resins, or the like and extrude the mixture as a thin ribbon as wide as pocket 11. The thickness of the ribbon should be sufficient to distribute in each unit volume of carbon in the plate 12 therebelow a predetermined quantity of lead iodide. The extruded ribbon is placed in pocket 11 and upon heating, the easily volatil-

ized binder evaporates before the lead iodide melts. For instance, polystyrene will depolymerize and the monomeric styrene will evaporate at temperatures of about 300° C. Thereafter the lead iodide left as a residue may be melted by heating to about 500° C.

The furnace atmosphere may be made neutral in order to prevent excessive oxidation of the brush or inadvertent oxidation or decomposition of the lead iodide or other halide compound. A gas secured by burning natural gas in air to a predetermined extent and characterized by substantially neutral properties is one type of atmosphere suitable for the purpose of this invention. Other atmospheres, for example, an all nitrogen atmosphere, may be introduced into the furnace 28 for the same purpose.

Since the carbon plates 12 are relatively thin, the process may be made more efficient by superimposing two or three or more plates with halide salt applied on the conveyor 14 for simultaneous treatment. The ledges 13 will provide for the proper spacing between each layer of plates. Separate spacers may be employed in case plates without ledges are being processed.

Measured amounts of halide salts may be applied manually or in other ways than shown in Fig. 1. Likewise, carbon plates with the salt applied to the upper surface thereof may be manually placed in an oven and removed when fully impregnated. It will be clear to those skilled in the art that other forms of apparatus may be employed to carry out the process disclosed. For instance, the plates may be pushed along a graphite trough into the furnace instead of being carried on the belt type conveyor shown in Fig. 1.

In some cases, instead of applying the salt in crystal form, the salt may be premelted and applied in a liquid state to the surface of the carbon plates previous to placing the plates in a furnace.

Other methods of depositing or applying the salt than by the measuring device to the brushes prior to the heat treatment have been found to be satisfactory. In some cases, a predetermined quantity of the salt made into a paste by adding a liquid thereto may be spread or brushed upon the upper surface of the brush and on entering the furnace the solvent or liquid carrier will be evaporated, leaving the dry salt in condition for melting and penetration of the carbon brush. The salt may be applied in any desirable physical state, since, when subjected to the high temperatures in the furnace, the salt will melt and impregnate the carbon body.

By applying a measured quantity of the salt to each individual brush, it will be apparent that there will be no question of whether or not each brush member has been given a satisfactory quantity of the iodide or bromide. Since it is quite important that each brush operate at the optimum efficiency, it is desirable that each brush have a minimum predetermined quantity of salt present therein.

Any type carbon electrode may be treated according to this invention, including graphitic brushes and metallic-carbon brushes. In practicing the process it has been found that graphitized brushes may be treated somewhat more satisfactorily than ungraphitized carbon. The graphitizing of carbon plates is believed to result in a greater porosity leading to a more rapid penetration and absorption of the salt. By comparison metallic-carbon brushes have been found

to absorb the salt very slowly and in lesser amounts.

Since certain changes may be made in the above invention, and different embodiments of the invention may be made without departing from the scope thereof, it is intended that all matter contained in the above disclosure or taken in connection with the accompanying drawings shall be interpreted as illustrative and not in a limiting sense.

I claim as my invention:

1. The process of impregnating a graphitized carbon brush with a metallic halide comprising applying a predetermined amount of the metallic halide to an upper surface of the brush and heat-treating the brush and applied solid halide to a temperature to melt the halide for a period of time sufficient to cause the molten halide to penetrate into or be absorbed by the brush thereby by securing a distribution of the metallic halide in the body of the brush.

2. The process of impregnating a carbon brush with a material capable of decreasing dusting and wear comprising applying a predetermined amount of a solid metallic halide material to a substantially horizontally disposed upper surface of the brush, and heating the brush and applied material to a temperature sufficient to melt the material and to cause the molten metallic halide material to penetrate into or be absorbed by the brush to provide for a predetermined distribution of the material throughout the brush.

3. The process of impregnating a carbon brush with a metallic halide, comprising forming a pocket in an upper surface of a porous carbon body to be used in preparing the brush, applying a predetermined amount of the metallic halide in the pocket in the body and heating the body and applied metallic halide to temperatures sufficient to melt the halide, the pocket serving to retain the molten halide, the heat treatment being for a period of time sufficient to cause the molten halide to penetrate the body and be absorbed thereby.

4. The process of impregnating carbon bodies with a metal halide comprising, in combination, mixing the metal halide with a binder which will evaporate below the melting temperature of the metal halide, forming the mixture into a ribbon having a predetermined weight of metal halide per unit area, applying the ribbon over a surface of the carbon body, and heating the ribbon to a temperature to cause the binder to evaporate and thereafter heating to a temperature to melt the

metal halide and to impregnate the carbon body.

5. In the process of incorporating a metallic halide in a porous carbon body, the steps comprising, disposing the porous carbon body in such position that an upper surface is substantially horizontal, applying to the substantially horizontal upper surface a predetermined amount of a solid metallic halide and heating the carbon body and applied metallic halide to a temperature high enough to melt the metallic halide.

6. In the process of incorporating in a porous carbon plate having substantially flat surfaces a metallic halide, the steps comprising, disposing a substantially flat upper surface of the carbon plate in a substantially horizontal plane, applying to the substantially flat upper surface a predetermined amount of solid metallic halide distributed relatively uniformly over the surface, heating the carbon body and applied metallic halide to a temperature high enough to melt the metallic halide, and continuing the heating until the molten metallic halide has penetrated into the pores of the carbon body and is distributed throughout the carbon body.

7. In the process of impregnating a carbon brush with a metallic halide salt, the steps of applying a quantity of the metallic salt to an upper surface only of the brush and heat-treating the brush and applied salt at a temperature at which the metallic salt will be molten and for a sufficient time so that it will penetrate the brush to provide for a predetermined distribution of the metallic salt in the brush.

LAWRENCE E. MOBERLY.

35

#### REFERENCES CITED

The following references are of record in the file of this patent:

#### UNITED STATES PATENTS

| Number       | Name     | Date          |
|--------------|----------|---------------|
| 1,000,761    | Snyder   | Aug. 15, 1911 |
| 1,184,135    | Rudolph  | May 23, 1916  |
| 1,626,104    | Swift    | Apr. 26, 1927 |
| 45 1,716,461 | Portail  | June 11, 1929 |
| 1,779,242    | Laube    | Oct. 21, 1930 |
| 1,861,415    | Hunter   | May 31, 1932  |
| 1,867,524    | Orne     | July 12, 1932 |
| 50 1,868,206 | Hunter   | July 19, 1932 |
| 1,895,756    | Fuller   | Jan. 31, 1933 |
| 1,620,940    | Bleecker | Mar. 15, 1927 |
| 1,742,259    | Kelleher | Jan. 7, 1930  |
| 2,098,062    | Palmer   | Nov. 2, 1937  |